

May 12, 1936.

U. B. BRAY ET AL

2,040,239

## PROCESS FOR PRODUCTION OF LUBRICATING OILS

Filed Feb. 13, 1934



## UNITED STATES PATENT OFFICE

2,040,239

PROCESS FOR PRODUCTION OF  
LUBRICATING OILS

Ulric B. Bray, Palos Verdes Estates, and Claude E. Swift, Glendale, Calif., assignors to Union Oil Company of California, Los Angeles, Calif., a corporation of California

Application February 13, 1934, Serial No. 711,026

7 Claims. (Cl. 196—13)

This invention relates to the process for treating petroleum to produce lubricating oil and is a continuation-in-part of our co-pending application Ser. No. 555,017, filed Aug. 4th, 1931.

5 It has been observed by one of us that many oils containing asphalt and wax are mixtures of hydrocarbons analogous both to hydrocarbons present in paraffin base oils and those present in asphalt base oils. It has been observed by one 10 of us, (Ser. No. 466,189), that during the heating of an oil containing asphalt that a reaction is set up whereby the inherent low viscosity temperature susceptibility of the lubricating oil fractions is destroyed.

15 In order to preserve the inherent characteristics of the lubricating oil components of crude oil containing asphalt which are impaired by distillation methods, we have, in accordance with the process of the above application, caused the separation of the oil and wax from the asphalt by a method wherein the lubricating oil constituents present in the crude oil are separated from the asphalt present in such a manner that the oil retains those characteristics which it possessed in 20 the original crude oil. As a means of attaining this, it has been found advisable to cause the separation of the asphalt from the oil by means of solvents which are capable of dissolving the oil and which do not dissolve the asphalt. Such 25 solvents are alcohol, ether, mixtures of alcohol and ether, acetone, etc., particularly naphtha, casinghead gasoline and petroleum fractions normally vaporous at ordinary temperature and pressure. We prefer to use as our solvent a petroleum

30 fraction which may be obtained by the rectification of natural gasoline. For some purposes a fraction composed of 6.72% ethane, 72.2% propane, 19.91% iso-butane and 1.17% normal butane is satisfactory. However, by using a fraction 35 containing a higher percentage of ethane, it is possible to produce a lubricating oil having a low Conradson carbon value. Such a solvent has a tendency to leave certain heavy oil fractions in the precipitated asphalt which have a tendency 40 to form a high carbon residue. Such a fraction suitable for the production of a lubricating oil having a low Conradson carbon value would contain ethane varying in quantities from 40 to 50% by volume.

45 It is the purpose of this invention to use this type of solvent to separate the asphalt from the oil, i. e. a solvent composed mainly of ethane and propane.

In carrying out the extraction of the oil with 50 this light liquid fraction, the solution is main-

tained at a pressure sufficient to maintain the solvent liquid. The extraction of the oil from the petroleum at such pressures to maintain the solvent liquid, results in an asphalt substantially free of oil compound chiefly of bitumen and a 5 solution of oil and wax in the liquid petroleum fraction. The oil dissolved in the solvent contains substantially all of the lubricating oil components which are present in the crude oil and in substantially the same form as they exist in the 10 original crude oil and also the major portion of the wax present in the crude oil.

One of the desirable qualities of a lubricating oil is a low Conradson carbon value. According to the U. S. Government Department of Commerce, 15 Bureau of Mines Technical Paper 323B, page 86, this value throws some light upon the relative carbon forming properties of an oil. Oils which possess a low value have less tendency to cause carbon deposition in internal combustion motors 20 during use than do oils which possess a high value. In general, lubricating oils produced by ordinary distillation processes from crudes containing asphalt exhibit a low Conradson carbon value, whereas lubricating oils produced from paraffin 25 base crudes exhibit high value.

It is one of the characteristics of the lubricating oil produced by our process that it possesses a low Conradson carbon value. In Table I, Conradson carbon values are shown for a typical 30 paraffin base lubricating oil, a typical asphalt base lubricating oil and a typical oil produced by our process.

TABLE I  
Conradson carbon values

|                                                                   | S. A. E.<br>grade | Conradson<br>carbon<br>values |
|-------------------------------------------------------------------|-------------------|-------------------------------|
| Paraffin base lubricating oil produced<br>from Pennsylvania crude | 40                | 0.80                          |
| Asphaltic base lubricating oil produced<br>from California crude  | 40                | 0.25                          |
| Oil produced by our process produced<br>from California crude     | 40                | 0.15                          |

Another desirable quality of lubricating oil is a high resistance towards oxidation. In general, 50 oils which oxidize less rapidly are to be preferred. Lubricating oils produced from paraffin base crudes have less tendency to oxidize than lubricating oils produced by the distillation of asphalt base crudes. It is one of the characteristics of the oil produced by our process from 55

asphalt base crudes containing wax that it possesses a low oxidation value.

One of the methods used to determine the oxidation value of an oil is to be found in the Proceedings of the American Society of Testing Materials, vol. 24, Part II of 1924, page 964, and is sometimes known as the Sligh method.

In Table II there is shown a comparison of the oxidation values of a lubricating oil produced from paraffin base crude, a lubricating oil produced by our process from asphalt base crudes containing wax, and a lubricating oil produced by the distillation of asphalt base crude:

15

TABLE II  
*Sligh oxidation values*

|                                                                              | Sligh oxidation value |
|------------------------------------------------------------------------------|-----------------------|
| Paraffin base lubricating oil produced from Pennsylvania crude               | 5.0                   |
| Asphaltic base lubricating oil produced by our process from California crude | 4.0                   |
| Asphaltic base lubricating oil produced from California crude                | 40.0                  |

It is thus an object of our invention to produce lubricating oils from asphalt containing oils having relatively low Conradson carbon values.

It is a further object of our invention to precipitate asphalt from an oil containing asphalt with a normally gaseous hydrocarbon solvent containing a large amount of ethane, preferably 40 to 50% ethane and the remainder largely liquid propane.

A further object of our invention is to commingle an oil containing wax with a solvent composed largely of ethane and propane, then separating a portion of the solvent in one stage and a further portion in a second stage under reduced pressure whereby the oil containing wax and remaining solvent is chilled to a sufficiently low temperature to enable wax to precipitate out of solution which is separated from the oil and solvent, after which the remaining solvent is separated from the oil.

Other objects and features of our invention will be apparent from the following description of our process taken from the drawing, representing a schematic arrangement of apparatus.

Referring to the drawing, crude oil from which all of the gasoline, kerosene and gas oil have been removed in tank 1 is withdrawn through valve 2 and sent by means of pump 3 to line 4 where it meets a stream of solvent under pressure, i. e. the mixture of ethane and propane referred to above coming from storage tank 11 through valve 12, pump 13 and line 14. The mixture of topped crude and solvent passes into chiller 5 where the mass is cooled by allowing a portion of the solvent to vaporize under reduced pressure through valve 6 into line 7. The vaporized solvent in line 7 is compressed by compressor 8 and sent to condenser 9 where it is liquefied and passes by means of line 10 to solvent storage tank 11.

The cooled mass of topped crude and solvent in chiller 5 passes by means of line 15 to agitator 16 where it is thoroughly mixed, after which it passes by means of line 17 to decanter 18 where the asphalt settles out.

The asphalt in decanter 18 is removed through valve 19 and sent by pump 20 through line 21 to heater 22 where the temperature of the mass is raised sufficiently to vaporize all the solvent and moisture present. The heated mass then passes by means of line 23 into separator 24 where the asphalt separates out and is removed through

valve 25 and line 26 to storage tank 27. The mixture of water and solvent vapors passes from separator 24 through line 28 to condenser 29 where the water vapor is condensed. The mixture of water and solvent vapor passes from condenser 29 to separator 30 where the water is separated out and is removed through valve 31 and line 32. The solvent vapor in separator 30 passes by means of line 33 to compressor 34 where it is compressed and sent by means of line 33' to condenser 9 where it is liquefied and passes through line 10 to storage tank 11.

The solvent solution of oil in decanter 18 is withdrawn through line 35 and passes into chiller 36 where the temperature of the mass is lowered to a point sufficient to cause thorough wax precipitation by allowing a portion of the solvent present in chiller 36 to vaporize under reduced pressure through valve 37 into line 38. The solvent vapor in line 38 is compressed by compressor 39 and sent through line 38' to condenser 9 where it is liquefied and passes by means of line 10 to storage tank 11.

The cooled mass in chiller 36 is withdrawn through valve 40 and line 41 whereafter it is sent by pump 42 to a dewaxing stage 43 which may consist in centrifuging, filtering or cold settling the chilled mass to remove the wax which is withdrawn via line 43'. The dewaxed oil dissolved in solvent emerges from the dewaxing stage into line 44 where it is mixed with sulphuric acid coming from tank 45 through valve 46, line 47, pump 48 and line 47'. The mixture of oil and acid then passes into agitator 49 where it is thoroughly mixed, after which it passes into decanter 51 where the sludge is allowed to settle out.

The sludge in decanter 51 is removed through valve 53 and sent by means of pump 54 through line 55 to heater 56 where the temperature of the mass is raised sufficiently to vaporize the solvent. The heated mass then passes by means of line 57 to separator 58 where the sludge separates out and is withdrawn through valve 59 and line 60. The solvent vapor passes from separator 58 through line 61 to scrubbing tower 62 where it is contacted with liquid caustic soda introduced through line 63 to remove any acid present, the caustic soda and impurities being withdrawn via line 65 and valve 64. The scrubbed solvent passes from tower 62 through valve 66, line 67, compressor 68, line 67' to condenser 9 where it is liquefied and passes by means of line 10 to storage tank 11.

The acid treated oil dissolved in solvent in decanter 51 passes by means of line 52 to clay tower 80 where any remaining sludge is removed. The solvent solution of treated oil then passes from tower 80 by means of line 69 to evaporator 70 where the solvent present is vaporized with the aid of steam introduced through closed steam coil 74. The solvent vapor passes from evaporator 70 through valve 71 into line 72 thence to compressor 73 where it is compressed and sent by means of line 72' to condenser 9 where it is liquefied and passes by means of line 10 to storage tank 11. The solvent-free oil in evaporator 70 is withdrawn through valve 75 and passes through line 76 into storage tank 77. If desired, this oil may be subjected to extraction with a selective solvent, such as liquid sulphur dioxide, for the purpose of separating the non-paraffinic fractions from the paraffinic oil. This portion of the process may be carried out according to the process

described in our co-pending application Ser. No. 555,017.

As illustrative of the operation of the process for one type of oil without intending to limit our 5 invention, the following is an example:

The topped oil in tank 1 at a temperature approximating 200° F. is mixed with solvent and cooled by allowing a portion of the solvent present to vaporize until a temperature of about 120° F. 10 is attained, after which the mixture of residual oil and solvent is mixed in agitator 17. The thoroughly agitated mass passes into decanter 18 where the solvent solution of oil and wax is separated from the undissolved asphalt. This oil 15 dissolved in solvent is chilled sufficiently to cause the wax present to precipitate out by allowing a further portion of the solvent present to vaporize under reduced pressure. The precipitated wax is removed from the solvent solution of oil by such 20 means as cold settling centrifuging or filter pressing. The oil substantially free of wax and asphalt dissolved in solvent is next treated with sulphuric acid introduced from tank 45. The result of this treatment is to remove further quantities 25 of undesirable bodies present in the oil which tend to give the finished product an increased viscosity temperature susceptibility. After treatment with the sulphuric acid, the oil is separated from the solvent and may further be refined by extraction with a selective solvent such 30 as liquid sulphur dioxide.

The foregoing exemplary description is merely illustrative of a preferred mode of carrying out our invention and is not to be taken as limiting 35 as many variations may be made within the scope of the following claims by a person skilled in the art without departing from the spirit thereof.

We claim:

40 1. A process for separating asphalt from oils containing the same which comprises commingling said oil with a liquefied normally gaseous hydrocarbon solvent containing propane and approximately 40% ethane to precipitate asphalt, 45 separating the precipitated asphalt from the oil and solvent and separating the solvent from the oil.

2. A process for separating asphalt from oils containing the same which comprises commingling 50 said oil with a liquefied normally gaseous hydrocarbon solvent containing propane and approximately 40% to 50% ethane to precipitate asphalt, separating the precipitated asphalt from

the oil and solvent and separating the solvent from the oil.

3. A process for separating asphalt from oils containing the same which comprises commingling said oil with a liquefied normally gaseous hydrocarbon solvent containing approximately 40% ethane and the remainder largely propane to precipitate asphalt, separating the precipitated asphalt from the oil and solvent and separating the solvent from the oil. 10

4. A process for the production of lubricating oil from oil containing wax which comprises commingling said oil in a light liquefied hydrocarbon solvent comprising a mixture containing propane and approximately 40% ethane, vaporizing a part 15 of the solvent in one stage and vaporizing another portion in a second stage to chill the oil and precipitate the wax, separating the precipitated wax from the remaining oil solvent solution and separating the remaining solvent from the oil. 20

5. A process for the production of lubricating oil from oil containing wax which comprises commingling said oil in a light liquefied hydrocarbon solvent comprising a mixture containing propane and approximately 40% to 50% ethane, vaporizing a part of the solvent in one stage and vaporizing another portion in a second stage to chill the oil and precipitate the wax, separating the precipitated wax from the remaining oil solvent solution and separating the remaining solvent 30 from the oil. 35

6. A process for the production of lubricating oil from oil containing asphalt and wax which comprises commingling said oil in a light liquefied hydrocarbon solvent comprising a mixture containing propane and approximately 40% ethane to precipitate asphalt, separating the precipitated asphalt from the oil, wax and solvent and separating the wax from the oil and solvent. 40

7. A process for the production of lubricating oil from oil containing asphalt and wax which comprises commingling said oil in a light liquefied hydrocarbon solvent comprising a mixture containing propane and approximately 40% ethane to precipitate asphalt, separating the precipitated asphalt from the oil, wax and solvent, chilling the oil and solvent to precipitate the wax, separating the precipitated wax from the oil and solvent and separating the solvent from the oil. 45 50

ULRIC B. BRAY.  
CLAUDE E. SWIFT.